

C. NAPIER.

**TEMPERED BLADE.**

APPLICATION FILED JAN. 30, 1919.

1,352,140.

Patented Sept. 7, 1920.



44 Inventor  
Charles Napier  
By Robert Roberts & Bushman  
his attorney.

# UNITED STATES PATENT OFFICE.

CHARLES NAPIER, OF SPRINGFIELD, MASSACHUSETTS, ASSIGNOR TO NAPIER SAW WORKS, INC., OF SPRINGFIELD, MASSACHUSETTS, A CORPORATION OF MASSACHUSETTS.

## TEMPERED BLADE.

1,352,140.

Specification of Letters Patent. Patented Sept. 7, 1920.

Original application filed December 9, 1918, Serial No. 265,836. Divided and this application filed January 30, 1919. Serial No. 274,006.

To all whom it may concern:

Be it known that I, CHARLES NAPIER, a citizen of the United States of America, and resident of Springfield, in the county of 5 Hampden and State of Massachusetts, have invented new and useful Improvements in Tempered Blades, of which the following is a specification.

This invention relates to cutting tools and 10 comprises a blade such as a saw, knife or other cutting implement having new and valuable characteristics.

In my Letters Patent No. 1,221,576, dated April 3, 1917, I have explained a machine for uniformly tempering saw-blades, and in my Letters Patent No. 1,265,944, dated May 14, 1918, I have explained a method of heat-treating such blades adapted to be carried out with the aid of such a 20 machine, the product of the later patent being a uniformly tempered blade with annealed or soft ends useful as a hack-saw and for other purposes. Such blades are first hardened and then draw-tempered throughout their middles and edges to the degree of 25 hardness or temper heretofore customary for such blades. This customary degree of temper is such, in the instance of the hack-saw, band-saw and other such blades, of prior knowledge, as to provide a moderately 30 flexible and resilient blade uniformly hard enough to enable any of its edges to serve as a metal-cutting edge, the finished blade proper, including the edge, being thus characterized by a uniform crystalline structure 35 with a low elastic limit, and therefore being brittle against sharp bending or sudden blows. In the best practice of which I am aware, I have collected statistics showing 40 that more than 42 per centum of hack-saw blades are broken in use before the usefulness of the cutting edge is impaired at all by wear. Such breakage represents a loss of value of a still higher figure if breakages 45 after a partial use of the tool should be included.

A principal object of the present invention is to avoid such losses of value by the

provision of a blade having a cutting edge of greater hardness than has heretofore been 50 practicable and a body which will not break under the ordinary strains of use.

Available tool-steels have heretofore necessitated for such uses a compromise between resilient flexibility and hardness, a 55 high elastic limit being attained by draw-tempering with any available material only upon treatment resulting in reducing the hardness of the metal below an attainable, and for metal-cutting purposes, the most 60 useful value or degree. For instance, it is my experience that a "glass-hard" state, attained by first heating to a high critical temperature and then chilling or quenching, is most useful for the edges, points or teeth of 65 a metal-cutting saw, knife, or milling cutter in respect to its attack upon the material; but it is also my experience that this state is impracticable for such an instrument as a saw-blade, because the desirable quality of 70 extreme hardness is accompanied by such brittleness and susceptibility to breakage in use as to limit unduly the life of the tool.

It has therefore been customary heretofore to sacrifice the quality of maximum 75 hardness in favor of an increased springiness and toughness, the blades being tempered by subjection to a moderate uniform heating after hardening so as to stand moderate bending without breakage, despite the fact 80 that this treatment reduces the extreme hardness of the cutting edge which it would have been advantageous to retain if there were any way to keep it compatible with securing toughness and resilience. When 85 hard enough to cut, the blade still remains so brittle as to require the most careful use.

I have discovered that a cutting edge of such a tool as a knife, band-saw or hack-saw blade may be kept at a point at or near its 90 maximum hardness, thereby to produce a cutting tool of heretofore unknown durability and efficiency, if the hard edges or portions are supported by intimate and integral contact with portions of the body of the 95 blade gradually decreasing in hardness and

increasing in resilience or softness within the hard points or edges. For instance, points or edge portions which have been heated above the hardening reaction point, quenched or chilled, [and if desired slightly draw-tempered to an extent not reducing the desired hardness for cutting at a low heat, about 350° F. for instance, for tool-steels of usual composition] may be supported upon integral bases or a backing of the same metal which has been first hardened and then drawn, as the edge is receded from, at temperatures varying with the extent of recession from the hard points or edges from about 350° to about 800° F., or such other temperature as will leave the article in a springy resilient state. Such a spring temper is a highly desirable quality of the blade proper of such an article, but it is not compatible with sufficient hardness for metal cutting, and is as detrimental at the ultimate cutting edge or point as it is valuable in the body of the tool.

I have also devised and have explained in my application Serial No. 265,836, filed December 9, 1918, of which this is a division, a method or art of rapidly, uniformly, and if desired, continuously treating such articles so as to provide them with hard cutting points or edges and with gradually and increasingly softer and more flexibly resilient supports but harder than the body of the blade for the point or edge and within the point or edge, and with substantially uniform spring-tempered bodies integral with and bearing such support and edge. As an article of manufacture, the resulting product retains the cutting quality of hard teeth or edges against long wear, and resists breakage remarkably. I shall herein describe as an instance of the genus of new articles characterized by my invention a hack-saw blade, and I shall also herein describe as one instance only of the method of heat-treating such a blade also constituting a part of my invention, steps specifically applicable to this particular article, but applicable without change except of apparatus or degree to the treatment of other specific articles included among the new genus of articles comprising my invention.

In the accompanying drawings,—

Figure 1 is a diagram elevation of a typical specimen of the article of manufacture;

Fig. 2 is an enlarged detail of the area 2-2 of Fig. 1;

Fig. 3 is a diagram section on line 3-3 of Fig. 2 illustrating graphically the relative hardness of the metal at different parts;

Fig. 4 is a diagram plan of preferred apparatus for practising the method;

Fig. 5 is an enlarged detail diagram in plan showing relationships of temperatures and previous conditions of the metal being treated; and

Fig. 6 is a detail section at the edge-heater showing one arrangement for differentially heating the parts of the article.

Referring now to Figs. 1, 2 and 3, if the instrument is a saw, a preferred state of the metal is that in which the blade 10 is substantially uniformly spring-tempered to a flexible resilience with a high elastic limit throughout the region 13 comprising the greater part of the body or blade; and in which the points, faces and cutting edges 15 of the teeth are of the maximum hardness compatible with enough tensile coherence to prevent chipping or shivering. At the ultimate faces, edges and points, this may be the maximum crystalline hardness which the metal is capable of assuming, such as will follow heating above the critical temperature [1200° to 1400° F. or higher, for tool steels of commercial composition] and immediate quenching at temperatures at or below 350° F.

If any considerable depth of the teeth or edges of the saw is in such a crystalline state, breakage under use is inevitable. For instance, if a whole tooth comprising the points and edges and faces 15 and the base or root 16 is in this state, breakage of that tooth under lateral strain or a sharp blow or bending of the blade at a moderate angle is to be expected. If the region 14 adjoining the teeth is glass hard, such a breakage may involve two or more teeth. But if only the faces and edges and points are of a crystalline hardness, if the roots or bases 16 are hard but tough, and if the region 14 back of the roots 16 partakes of the qualities of resilience and flexibility, breakages of teeth do not occur. Desirably, then, the hard points and faces 15 and the spring-tempered body 13 are separated by a region 14 partaking of the qualities of the hard parts at these parts, and of the quality of the springy part at the juncture at line *a* of the blade, which may be near the toothed or cutting edge. I have found that the best results for efficiency and durability are attained when the region 13 is uniformly spring-tempered and when the region 14 increases in hardness from uniformity with the temper of region 13 from the line *a* toward the toothed edge. As shown graphically in Fig. 3, a curve *a* whose ordinates represent hardness at abscissæ successively approaching the edge rises to a maximum at the edge.

Preferably the blade is of the kind provided with perforations 11 at each end and with soft or annealed regions 12 at the neighborhood of the perforations, responding in this respect to the product of the art or method set out in my said Letters Patent No. 1,265,944. The blade proper, comprising the regions 13 between the regions 12, 12, and the edge region 14 has first been sub-

jected to heating above a critical temperature dependent on the material [for instance to the cherry-red hardening temperature for tool steels of usual carbon contents adapted to

5 take a hardening reaction at the cherry-red temperature]; has been thereafter subjected to sudden cooling, as in an oil-bath; and the region 13 only has been tempered by subjection to a temperature in a neighborhood 10 of 800° F., more or less, in accordance with the reaction of the particular metal under treatment at the hardening stage.

The region 14 and the faces, edges and points 15 have been subjected to steps first 15 hardening these regions uniformly; then heating them above the temperature for hardening reaction; then chilling or quenching; and then "drawing the temper" of the region 14 and the bases of the teeth, points or 20 edges by regulated causation of temperatures decreasing toward the edges or points and acting during a predetermined time only, the effect being to spring-temper the part of the strip or region 14 at its juncture with 25 the spring-tempered blade, and to leave unaffected the condition attained at the edges or points when the edge containing them was quenched or chilled. Preferably the quenching of the edge strip 14 was so conducted as to occur at a regulated minimum 30 temperature consonant with drawing the temper of the inner side of the strip and the inner parts of the metal blade during maintenance of this temperature at the 35 chilled faces, edges and points.

These qualities of the product will best be understood by explanation of a specific preferred instance of the steps taken in making 40 on a commercial scale articles of the kind referred to.

Referring now to Figs. 4, 5 and 6, the process is preferably practised continuously by subjection of a series of the articles to be treated successively during predetermined 45 times to the different stages of treatment. A convenient way to do this to provide for joining the articles end to end in a chain and to move them forward, for instance by such means as disclosed in my said Letters Patent No. 1,221,576, dated April 3, 1917, at a constant rate (either intermittently by short steps or continuously) past heating, quenching, reheating, tempering, cooling and washing devices suitable to the particular result 55 desired; but it will be understood that any desired means for subjecting the articles in succession to the described stages of treatment may be employed. A preferred process is described and claimed in my said application S. No. 265,836, filed Dec. 9, 1918, 60 of which this application is a division.

The individual articles 10 first pass through a gas-heated muffle-furnace 20 in which the articles 10 and their connectors 9 65 are heated uniformly. Preferably the arti-

cles, if for saws, are of steel of one of the following typical analyses:

*Carbon steel.*

|            | Percentages. |      | 70 |
|------------|--------------|------|----|
|            | Min.         | Max. |    |
| Carbon     | 1.05         | 1.10 |    |
| Manganese  | .20          | .30  |    |
| Sulfur     | .015         | .08  | 75 |
| Phosphorus | .015         | .09  |    |
| Silicon    | .035         | .045 |    |
| Nickel     | .003         | .006 |    |

*Tungsten steel.*

|            | Percentages. |      | 80 |
|------------|--------------|------|----|
|            | Min.         | Max. |    |
| Tungsten   | 1.10         | 1.25 |    |
| Manganese  | .20          | .30  | 85 |
| Sulfur     | .010         | .08  |    |
| Phosphorus | .010         | .09  |    |
| Silicon    | .010         | .015 |    |
| Carbon     | 1.10         | 1.20 |    |
| Nickel     | .00          | .003 |    |

In either cases a temperature at muffle 20 of from 1350° to 1400° F. is satisfactory, and this is readily attained during progress of the saws at about 14 feet a minute through a hot passage about three feet long.

From the muffle the saws pass to a quenching tank 30 in which a suitable liquid, such as an oil or emulsion at about 100° F. chills the saws to a uniform glass-hard state, except at the ends, which are prevented from rapid cooling by the mass of holders 9, and 100 remain soft.

The saws now pass into a heater 40 in which the blades are heated to about 800° to 850°, to draw the temper of the region 13 to a spring-temper, and to heat the edge 105 strip 14, 15, again to a red heat at 1400° or more. Preferably a metal block 41 channeled at 42 to receive all of the saw-blades except the strip 14, 15, is positioned to receive a predetermined length of the traveling chain of saws. Heater 40 may comprise a block 41 and a refractory screen 43 supported on a base 44, and adjustable gas-blasts 45 playing downward upon the exposed edge strips 14 and the block 41. By 110 proper regulation of the length and mass of the block 41, the intensity, temperature and number of the gas-blasts 45, no difficulty is found in maintaining the relative temperatures of the regions 13 and 14 of the saws 120 at exit from the heater 40 at the desired figures, which are near or slightly in excess of 800° and 1400° F. respectively for the body and edge strip, as indicated in Fig. 4. The block 41 may be about ten inches long 125 for an article-chain speed of 14 feet a minute. Saws which were cool and glass-hard before entering heater 40 thus leave it differentially heated to degrees adapted to cool slowly to a spring temper and to chill to 130

130

hardness respectively at the regions 13 and 14.

The heated blades are then subjected to treatment at a bath 50 adapted to resist too rapid cooling of the region 13; and first to quench or chill the strip 14 and the faces, edges and points at the edge 15, and thereafter to permit the residual heat of the body 13 and strip 14 to effect a predetermined drawing of the temper of the strip 14. A preferred treatment comprises subjecting the hot running chain of blades to the action of a stream of high flash-point oil from a nozzle 51 at a temperature near 350° F., the oil being so delivered as to cling to and follow the chain for a predetermined distance, representing a time during which there is exchange of heat by conduction between the body 13 and the bath of hot oil, and during which the heat of the body 13 and strip 14, except the edges and points, falls to or near to the temperature of this bath. The very hot strip 14, and especially the edges, faces and points 15 fall to this temperature so rapidly as to harden the cutting edges to the desired maximum degree; but the region 13 does not harden. I have discovered that there is a sufficiently rapid drop of temperature at the points and edges from red heat toward the temperature of the hot oil bath to carry out this reaction; that in a bath as described at or near 350° the tempering reaction at parts which have been heated only to a moderate temperature near 800° continues to the improvement of resilience and flexibility, and that a spring temper is under these conditions communicated progressively from region 13 into strip 14 to a degree depending on the time the conditions remain as indicated in bath 50. I ascribe the observed phenomena to the action in bath 50 after the quenching of the edge 14 of the residual heat of the greater mass of metal, *i. e.*, of the body 13 of the blades, since I find the distribution of hardness in the strip 14 to depend on the distance along the running chain [and hence on the time] during which the hot stream in bath 50 is allowed to act. The depth inward from the faces, edges and points 15 at which the metal is at maximum hardness varies inversely as this distance, so that the longer the immersion and the time taken at this stage, the shallower will be the hardest parts. The times involved are relatively short, a period of about two seconds in the hot bath being sufficient for hack-saws less than  $\frac{3}{2}$  inch thick.

The apparatus shown provides a cold bath 60 adjustable toward and away from the nozzle 51 so as to limit the time of immersion in the hot oil to produce the desired effect. Bath 60 may comprise a screen

61 to stop the hot oil stream, and may contain an oil or emulsion at 100° F. or less.

Bath 60 is long enough to reduce the saws approximately to its own temperature. After passing bath 60 the saws may pass through any desired form of wash-tank containing a hot alkaline washing solution, after which the saws are separated from the chain, and packaged for sale.

Particular attention is called to the characteristic of my new tool consisting of a region of graduated hardness greater than that of the blade or body and less than that of the cutting edges, points or faces, by the employment of which I provide for supporting the cutting edge, point or face on a flexible, resilient blade with a minimum liability to breakage from the blade or deformity of position with respect to the blade.

When I speak of the degree of temper or hardness of blades such as shown, it will be understood that I refer to a typical or average median longitudinal plane flatwise of the blade, and that the lateral faces of any typical blade according to my invention at any part of the region 14 may be of a graduated hardness decreasing inwardly from the edge less rapidly than the decrease of hardness of the typical median plane within the substance of the blade.

In some cases it will be understood that the lateral faces only of the blade at the region 14 may be at substantially maximum hardness, so long as the interior substance at the region 14 and between these faces possesses the described characteristic graduated decrease from maximum hardness to spring temper as the edge or face of the blade is receded from.

What I claim is:

1. A blade having a hardened cutting edge and a body integral therewith and in a state of spring temper, joined by an edge region gradually varying in hardness between said states, whereby the hard but brittle edge is supported against permanent bending and breakage upon a strip of metal at least as hard as the body of the blade, and decreasing in hardness as the edge is receded from.

2. An elongate flat blade having a hard cutting edge, an edge-region less hard, and a body tempered to a state of resiliency and not harder than any portion of said edge-region throughout its length.

3. A cutting-tool blade having a body uniformly spring-tempered, an edge having a cutting portion of maximum hardness, and a region between edge and body varying gradually from the hardened state of the edge to the spring temper of the body, and nowhere softer or more flexible than the body.

4. A spring-tempered saw blade charac-

terized by teeth whose edges, points and faces are in a state of maximum hardness, and by a narrow region harder and less flexible than the body of the blade for supporting the hard parts, said region varying gradually from the hard state of the edge to a state of spring temper at the juncture of said region with the body of the blade.

5. A saw blade having the cutting portions of one longitudinal toothed edge in a glass-hard state, the body of the blade back of said edge being tempered to a resilient flexible state, and having a region between body and edge harder and less flexible than 10 the body throughout, varying in temper from a springy state at its juncture with the body to glass-hardness near the points, faces

and edges of the teeth, and adapted to support the toothed edge against breakage in use.

6. A steel saw blade characterized by a body-portion tempered to a state of flexible resiliency, and by teeth having points, faces and edges in a state of crystalline hardness, the metal of the teeth and of the region at 25 the toothed edge of the blade gradually, as the edge is receded from, varying in temper from the hardness of the faces, points and edges to the same state as the body of the blade.

Signed by me at Springfield, Mass., this 30 twenty-seventh day of January, 1919.

CHARLES NAPIER.